

April 27, 1926.

1,582,673

F. A. FAHRENWALD

RIFLE BULLET

Filed May 21, 1924



Fig. 1



Fig. 2

Frank A. Fahrenwald

Inventor

by Smith and Freeman

Attorneys

## UNITED STATES PATENT OFFICE.

FRANK A. FAHRENWALD, OF CLEVELAND HEIGHTS, OHIO.

## RIFLE BULLET.

Application filed May 21, 1924. Serial No. 714,814.

*To all whom it may concern:*

Be it known that I, FRANK A. FAHRENWALD, a citizen of the United States of America, and a resident of Cleveland 5 Heights, in the county of Cuyahoga and State of Ohio, have invented certain new and useful Improvements in Rifle Bullets, of which the following is a full, clear, and exact description.

This invention relates to fire arms and especially to projectiles for use with high pressure, high velocity rifles. The objects of the invention are the provision of a new and improved bullet capable of velocities from 10 2500 feet to 3500 feet per second, which shall not strip in the bore or fuse at the base, nor break and disintegrate upon impact, nor seriously abrade the rifle barrel; the provision of a rifle projectile which can be made 15 in one piece and without jacketing; the provision of a rifle projectile which shall possess approximately the weight of lead but without the hardness of the customary jackets; the provision of a cheaper and better 20 bullet; while further objects and advantages 25 of the invention will become apparent as the description proceeds.

During the period when black powder was used and the velocities did not exceed about 30 1500 feet per second, a plain lead bullet or a bullet of lead hardened with a small amount of tin was perfectly satisfactory. With the advent of high pressure smokeless powders and the accompanying high velocities, this 35 plain lead or lead-alloy bullet could not be used since its softness caused it to become stripped in the bore instead of following the rifling, the high temperature of the gases partially fused it at the base, and the force 40 of impact was so terrific that even in soft animal tissues the bullet would fly into an infinite number of small pieces, sometimes even seeming to become vaporized. To overcome these defects the lead was jacketed 45 with a harder, tougher and more refractory material, a lead core still being used because of its high density, but this arrangement is unsatisfactory for large game shooting since with a strong jacket the bullet 50 merely pierces the target or animal, puncturing a clean-cut, small-diameter opening with very little stopping power. Many modifications of this jacketed bullet have been made, such as to expose the lead core 55 at the point or provide a small cavity inside the jacket near the point, with the object of

causing the bullet to mushroom, thus delivering to the game animal or other target the entire energy of the bullet and producing a more serious wound. Most bullets of this 60 type, however, fly into many pieces and are not nearly so effective as some of the lower velocity, softer bullets which merely spread out upon impact without becoming completely disrupted. 65

I have discovered that a bullet made of pure copper and thoroughly annealed after forming, behaves at high velocity (that is at velocities above about 2500 feet per second) in exactly the same manner as does a 70 lead bullet at the former velocity of 1500 feet per second. Being extremely soft and uniform it does not injure the bore of the finest rifle; being extremely tough and ductile it cannot strip but engages the grooves 75 very closely; its melting point is high enough to prevent fusion at the base no matter what the pressure or temperature of the driving gas; it is so soft and at the same time so tough and ductile that it produces a 80 typical mushroom upon impact and without disintegration.

Its specific gravity is slightly less than that of lead, being approximately 9.0 as 85 against approximately 11.25, yet the average density of a steel jacketed bullet is decreased by the fact that the steel jacket has a density of only about 7.6. As a result the weight of a copper bullet is less than 10% smaller than that of a steel jacketed bullet of equal size 90 which disparity can easily be made up by lengthening the bullet and without any observable effect upon the firing qualities or accuracy of the arm with which it is used since these longer copper bullets seem to 95 travel with the same trajectory as a shorter lead bullet of the same weight.

If desired to increase the stability of the bullet it is possible to use rifles with a slightly quicker twist inasmuch as the toughness of the copper will permit this to be done; although I have had most excellent results by the use of annealed copper bullets 100 in standard arms.

The cost of producing these bullets is less 105 than that for jacketed bullets. It is essential that very pure copper be used and that the same be thoroughly annealed after the final operation; or at least that very little deforming be effected after the annealing. 110 These bullets can best be formed by rolling pure copper into the form of rods, cutting

the rods into pieces of requisite length and forming these pieces in dies to the shape required. These bullets are then annealed, for example, by being maintained for five minutes at a temperature of 1400° F. I do not restrict myself as regards either the time or temperature of this annealing since a shorter time at a high temperature will serve equally well as a longer time at a lower temperature; it is essential that some annealing be done since cold swaged copper is hard, brittle, flies to pieces on impact, injures the rifling, and will not mushroom. If this annealing be carried out in a non-oxidizing atmosphere the bullets will issue with a bright polished appearance; by annealing in an oxidizing atmosphere or one containing sulphurous gases, it is possible to produce blackened bullets.

20 In the drawings accompanying and forming a part of this application Fig. 1 is an elevation and Fig. 2 a longitudinal sectional

view of one of my improved bullets. 1 represents the body of the bullet which is preferably made of a size to fit exactly the rifle lands, the base portion being preferably formed with one or more circumferential ribs 2 of a thickness approximately equal to the depth of the rifling. When used the numbers of these ribs may well vary with the length of the bullet, and be enclosed in the mouth of the shell (not shown). Owing to the extreme softness of the annealed copper these are not necessary as the body itself conforms so readily to the rifling.

Having thus described my invention what I claim is:

A one-piece bullet for high velocity rifles made of a single piece of substantially pure copper and annealed after fabrication.

In testimony whereof, I hereunto affix my signature.

FRANK A. FAHRENWALD.